

# United States Patent [19]

Rantell et al.

[11] 3,902,908

[45] Sept. 2, 1975

[54] **CATALYST SYSTEM FOR ACTIVATING SURFACES PRIOR TO ELECTROLESS DEPOSITION**

3,650,913 3/1972 D'Ottavio ..... 204/30  
3,698,919 10/1972 Kuzmik ..... 204/30 X

[75] Inventors: **Alan Rantell**, London, England;  
**Abraham Holtzman**, Bat-Yam,  
Israel

*Primary Examiner*—Lewis T. Jacobs  
*Attorney, Agent, or Firm*—Steward & Steward

[73] Assignee: **MacDermid Incorporated**,  
Waterbury, Conn.

## [57] ABSTRACT

[22] Filed: **Oct. 4, 1973**

An electroless metal plating catalyst and a particular method of preparing it at elevated temperature by reaction of a stannous salt and palladous or other similar catalytic metal ion augmented by incorporating a booster compound are disclosed. The resultant catalyst is useable at much lower catalytic metal concentration in plating operations than conventional prior catalysts. The booster compounds employed are acid or alkali soluble metal salts forming a sparingly soluble compound when contacted with conventional alkali or acid accelerators in the plating process.

[21] Appl. No.: **403,502**

### [30] Foreign Application Priority Data

Mar. 21, 1973 United Kingdom ..... 13545/73

[52] U.S. Cl. ..... **106/1; 117/47 A; 204/30**

[51] Int. Cl.<sup>2</sup> ..... **C23C 3/00**

[58] **Field of Search** ..... 106/1; 204/30; 117/47 A;  
252/441

### 8 Claims, No Drawings

### [56] References Cited

#### UNITED STATES PATENTS

3,532,518 10/1970 D'Ottavio ..... 204/30 X

**CATALYST SYSTEM FOR ACTIVATING SURFACES PRIOR TO ELECTROLESS DEPOSITION**

**CROSS REFERENCE TO PRIOR RELATED APPLICATIONS**

This application corresponds to British Provisional Specification No. 13545/73, filed Mar. 21, 1973.

**FIELD OF THE INVENTION**

The present invention relates to the preparation and use of a catalyst composition for activating non-conductive surfaces prior to electroless deposition of metals.

For the purpose of electroless or chemical plating of non-conductive substrates, small quantities of activator or catalyst must first be placed on the surface of the substrate. Palladium is found to be the most satisfactory catalyst but any metal selected from palladium, gold, silver or the platinum group of metals is suitable.

The activating or catalyzing process is often carried out by consecutive immersion of the substrate in solutions containing  $\text{PdCl}_2$  and  $\text{SnCl}_2$  respectively. More recently the use of single step activators comprising colloidal mixtures of  $\text{PdCl}_2$  and  $\text{SnCl}_2$  has been proposed. Typical working strength catalyst solutions contain:

|                                                     |                 |
|-----------------------------------------------------|-----------------|
| $\text{PdCl}_2$                                     | 300 – 1000 mg/l |
| $\text{SnCl}_2$                                     | 15 – 50 g/l     |
| $\text{Na}_2\text{SnO}_3 \cdot 3\text{H}_2\text{O}$ | 1 – 7 g/l       |
| HCl                                                 | 250 – 300 ml/l  |

However, these  $\text{PdCl}_2/\text{SnCl}_2$  mixtures are more effective when used in conjunction with an additional treatment solution known as an accelerator. Accelerators are generally solutions of strong acids or strong alkalies and are employed between the catalyst treatment and electroless deposition.

The method and conditions of preparation of  $\text{PdCl}_2/\text{SnCl}_2$  mixtures is critical. Further, the high concentration of  $\text{PdCl}_2$  employed makes the catalyst solutions very expensive. Less critical yet cheaper solutions would be an advantage.

**SUMMARY OF THE INVENTION**

The principle of the invention involves the formation of a highly active compound by reaction at high temperature between a stannous salt, usually the chloride, and low concentrations of palladous or other similar catalytic ions; e.g.  $\text{Au(I)}$ ,  $\text{Au(III)}$ ,  $\text{Pt(II)}$ ,  $\text{Pt(IV)}$ ,  $\text{Rh(III)}$ ,  $\text{Ru(III)}$ ,  $\text{Ru(IV)}$ ,  $\text{Os(III)}$ ,  $\text{Os(IV)}$ ,  $\text{Ir(III)}$ ,  $\text{Ir(IV)}$  or  $\text{Ag(I)}$ . The choice of booster compound is determined by the nature of the accelerator solution employed in the processing cycle. It is essential that the booster compound should form a sparingly soluble compound when contacted with the accelerator; i.e. if a  $\text{NaOH}$  accelerator is employed, the booster compound should be an acid salt of metal ion forming insoluble hydroxides at alkaline pH values; e.g. compounds containing  $\text{Mg}^{2+}$ ,  $\text{Fe}^{2+}$ ,  $\text{Fe}^{3+}$ ,  $\text{Mn}^{2+}$ ,  $\text{Cu}^{2+}$ ,  $\text{Ni}^{2+}$ ,  $\text{Co}^{2+}$  or  $\text{Cr}^{3+}$ .

In one method of implementing the present invention, the catalyst is formed by heating the component supplying the catalytic ion and the booster compound in strong acid solution at temperatures in excess of 75°C, and then adding an excess of stannous ion. The temperature of the mixture is maintained above 75°C

until the reaction is completed. During the reaction, the color of the mixture changes from light amber to dark brown, returning to light amber. Finally the completion of the reaction is indicated when the color of the mixture becomes dark brown for the second time. This may take from 1 to 20 minutes.

Alternatively the stannous ion may be added in two stages. Sufficient stannous salt to carry out the reaction is first added to the mixture of catalytic ion and booster compound at temperatures in excess of 75°C. The quantity required may be between 2 and 50 g/l as  $\text{SnCl}_2$  depending on temperature and concentration of catalytic ion. When the reaction is complete after 1–20 minutes, a vast excess of an acid stannous salt is added. Small quantities of sodium stannate are found useful for stabilizing the compound formed between  $\text{Sn(II)}$  and the catalytic ion, e.g.  $\text{Pd(II)}$ .

The preheating of the reactants to temperatures in excess of 75°C prior to admixing them in the preparation step is an important part of the invention. The catalytic activity of the reaction product formed between  $\text{Sn(II)}$  and the catalytic ion, e.g.  $\text{Pd(II)}$ , increases with increase of reaction temperature during manufacture, allowing relatively low concentrations of catalytic ion to be used. At temperatures below 75°C much greater concentrations of catalytic ion are required in order to maintain catalytic activity; viz. greater than 150 mg/l of  $\text{PdCl}_2$ . The reaction between  $\text{Sn(II)}$  and  $\text{Pd(II)}$ , i.e. the catalytic ion, may take two routes. The preferred reaction yields a  $\text{Sn(II)}/\text{Pd(II)}$  addition compound whereas a secondary reaction causes formation of metallic palladium. The latter reaction is generally undesirable. The use of high manufacturing temperatures and excess stannous salt encourages the preferred reaction and inhibits the secondary reaction.

The invention is illustrated by the following examples for the preparation and use of the catalyst.

**EXAMPLE I**

40 For 1 liter of working strength catalyst a mixture containing:

|                      |         |
|----------------------|---------|
| $\text{PdCl}_2$      | 45 mg.  |
| $\text{MnCl}_2$      | 15 g.   |
| HCl (37% w/v)        | 200 ml. |
| $\text{H}_2\text{O}$ | 400 ml. |

is heated to 90°C and reacted with a solution containing:

|                                                     |         |
|-----------------------------------------------------|---------|
| $\text{SnCl}_2 \cdot 2\text{H}_2\text{O}$           | 150 g.  |
| $\text{Na}_2\text{SnO}_3 \cdot 3\text{H}_2\text{O}$ | 4 g.    |
| HCl (37% w/v)                                       | 300 ml. |

55 The temperature is maintained at 90°C for 15 minutes and then allowed to cool prior to use.

The catalyst may be used to activate plastic surfaces or copper clad printed circuit boards prior to electroless deposition. For the plating of ABS plastics the following processing cycle is preferred:

60 ABS plastic is etched in a mixture containing 200–400 g/l  $\text{CrO}_3$  and 300–600 g/l  $\text{H}_2\text{SO}_4$  at 40°–70°C for 2–10 minutes. After thorough rinsing, the plastic is immersed in the catalyst solution for 1–5 minutes at room temperature. For increased activation it is permissible to heat the catalyst solution to temperatures up to 60°C. After further rinsing, the plastic is immersed in an accelerator solution containing 20–100

g/l NaOH for 1-5 minutes at 20°-60°C. The preferred temperature of the accelerator is 40°C. The activated plastic is then immersed in any electroless nickel or copper plating solution. A preferred composition is:

|                                                 |        |
|-------------------------------------------------|--------|
| NiSO <sub>4</sub> 6H <sub>2</sub> O             | 15 g/l |
| NH <sub>4</sub> Cl                              | 30 g/l |
| Na <sub>2</sub> H <sub>2</sub> PO <sub>4</sub>  | 60 g/l |
| pH adjusted to 8.0 - 8.5 with NH <sub>3</sub> . |        |

10

The electroless nickel solution is employed at 20°-30°C for 5-10 minutes.

### EXAMPLE 2

For 1 liter of working strength catalyst a mixture containing:

|                   |         |
|-------------------|---------|
| PdCl <sub>2</sub> | 45 mg.  |
| FeCl <sub>3</sub> | 40 g.   |
| HCl (37% w/v)     | 200 ml. |
| H <sub>2</sub> O  | 400 ml. |

is heated to 90°C and then reacted with 20g SnCl<sub>2</sub>·2H<sub>2</sub>O. After the reaction has continued for a period of 15 minutes, a mixture containing:

|                                                     |         |
|-----------------------------------------------------|---------|
| SnCl <sub>2</sub> ·2H <sub>2</sub> O                | 100 g.  |
| Na <sub>2</sub> SnO <sub>3</sub> ·3H <sub>2</sub> O | 4 g.    |
| HCl (37% w/v)                                       | 250 ml. |

30

The time allowed for the reaction of the first addition is not critical and may be for any period greater than 1 minute, but 15 minutes is preferred. The reaction temperature again is important, as it must be greater than 75°C, 90°-95°C being preferred.

The catalyst solution may be used to activate plastic surfaces in the manner described in Example 1.

### EXAMPLE 3

The catalyst is prepared and used as in Example 1 except that in this instance the PdCl<sub>2</sub> is replaced by 75 mg of HAuCl<sub>4</sub>.

### EXAMPLE 4

For 1 liter of working strength catalyst a mixture containing:

|                   |         |
|-------------------|---------|
| PdCl <sub>2</sub> | 40 mg.  |
| AlCl <sub>3</sub> | 20 g.   |
| HCl (37% w/v)     | 200 ml. |
| H <sub>2</sub> O  | 400 ml. |

40

is heated to 90°C and reacted with a solution containing:

|                                                     |         |
|-----------------------------------------------------|---------|
| SnCl <sub>2</sub> ·2H <sub>2</sub> O                | 150 g.  |
| Na <sub>2</sub> SnO <sub>3</sub> ·3H <sub>2</sub> O | 4 g.    |
| HCl (37% w/v)                                       | 300 ml. |

50

The temperature of the mixture is maintained at 90°C for 15 minutes and then cooled to room temperature for use. The electroless plating procedure then proceeds in a similar manner to that described in Example 1, except that in this instance the accelerator solution should be 10-500 ml/l of ammonia solution (28% w/v).

In this example AlCl<sub>3</sub> acts as a booster compound when used in conjunction with an ammonium hydrox-

ide accelerator since Al(OH)<sub>3</sub> is not soluble in ammonia solution.

### EXAMPLE 5

For 1 liter of working strength catalyst a mixture containing:

|                   |         |
|-------------------|---------|
| PdCl <sub>2</sub> | 45 mg.  |
| BaCl <sub>2</sub> | 40 g.   |
| HCl (37% w/v)     | 200 ml. |
| H <sub>2</sub> O  | 400 ml. |

is heated to 90°C and reacted with a solution containing:

|                                                     |         |
|-----------------------------------------------------|---------|
| SnCl <sub>2</sub> ·2H <sub>2</sub> O                | 150 g.  |
| Na <sub>2</sub> SnO <sub>3</sub> ·3H <sub>2</sub> O | 4 g.    |
| HCl (37% w/v)                                       | 300 ml. |

20 The temperature of the mixture is maintained at 90°C for 15 minutes and then the catalyst is cooled at room temperature for use.

25 The catalyst solution may be used to activate plastic surfaces in a similar manner to that described in Example 1, except that in this instance the accelerator solution should be 10-200 g/l H<sub>2</sub>SO<sub>4</sub>.

The activated catalysts referred to in the invention are not colloidal in nature. Tyndall effect measurements taken on the undiluted catalyst solutions and electron microscopy of the adsorbed catalyst fail to show any colloidal particles. The active component of the SnCl<sub>2</sub>/PdCl<sub>2</sub> catalyst is an acid soluble complex formed between Sn(II) and Pd(II). On contact with the accelerator solution, a slow redox reaction occurs:



The elemental palladium formed can then initiate electroless deposition. The presence of the booster enables a concentration of catalytic metal ion in solution equivalent to about 10 mg/l of Pd<sup>2+</sup> as PdCl<sub>2</sub> to be effective. For economic reasons a concentration equivalent to about 500 mg/l of PdCl<sub>2</sub> represents a practical maximum.

Booster compounds such as MnCl<sub>2</sub> and FeCl<sub>3</sub> produce a voluminous surface precipitate when the adsorbed catalyst contacts the sodium hydroxide accelerator. The precipitated metal hydroxides help to retain the Pd(II) on the plastic surface until the redox reaction has occurred. If no booster compound is used the Pd(II) may leach into the accelerator before any reaction has occurred.

What is claimed is:

1. A method for preparing a catalyst solution by heating an acid solution of a Pd(II) catalytic ion wherein said catalytic ion is present in amount sufficient to provide in the working strength catalyst solution a concentration equivalent to about 10-500 mg/l of Pd<sup>2+</sup> as PdCl<sub>2</sub>, with a solution containing a stoichiometric excess of stannous salt wherein at least one of said catalytic ion and stannous salt solutions is first heated to a temperature in excess of 75°C before the other is added to it, and wherein a booster compound consisting of a soluble metal salt, of which the cation is capable of forming a precipitate when contacted with the accelerator solution used in an electroless plating process, is added to the catalyst mixture during preparation, said booster compound being present in amount of about 0.1 mol/l up to 5 mol/l in the working strength solution.

2. A method for preparing a catalyst as in claim 1, for use in an electroless plating process employing as the accelerator a strong alkali, wherein the booster compound is a salt containing a cation selected from the group consisting of  $Mg^{2+}$ ,  $Fe^{2+}$ ,  $Fe^{3+}$ ,  $Mn^{2+}$ ,  $Mn^{3+}$ ,  $Cu^{2+}$ ,  $Ni^{2+}$ ,  $Co^{2+}$ ,  $Cr^{3+}$ .

3. A method for preparing a catalyst as in claim 1, for use in an electroless plating process employing as the accelerator an alkaline ammonia solution, wherein the booster compound is a salt containing a cation selected from the group consisting of  $Mg^{2+}$ ,  $Fe^{3+}$ ,  $Mn^{2+}$ ,  $Mn^{3+}$ ,  $Cr^{3+}$ ,  $Pb^{2+}$ ,  $Al^{3+}$ .

4. A method for preparing a catalyst as in claim 1, for use in an electroless plating process employing as the accelerator sulphuric acid or a soluble acid sulphate, wherein the booster compound is a salt containing a cation selected from the group consisting of  $Ca^{2+}$ ,  $Ba^{2+}$ ,  $Sr^{2+}$ ,  $Pb^{2+}$ .

5. A method for preparing a catalyst as in claim 1, for use in an electroless plating process employing as the accelerator a soluble carbonate or phosphate, wherein the booster compound is a salt containing a cation selected from the group consisting of  $Ca^{2+}$ ,  $Ba^{2+}$ ,  $Sr^{2+}$ ,  $Pb^{2+}$ ,  $Mg^{2+}$ ,  $Fe^{2+}$ ,  $Fe^{3+}$ ,  $Mn^{2+}$ ,  $Mn^{3+}$ ,  $Cu^{2+}$ ,  $Ni^{2+}$ ,  $Co^{2+}$ ,  $Cr^{3+}$ ,  $Cd^{2+}$ ,  $Zn^{2+}$ ,  $Pb^{2+}$ ,  $Al^{3+}$ .

6. A method for preparing a catalyst as in claim 1, for use in an electroless plating process employing as the accelerator a soluble fluoride, wherein the booster compound is a salt containing a cation selected from the group consisting of  $Mg^{2+}$ ,  $Ca^{2+}$ ,  $Ba^{2+}$ ,  $Sr^{2+}$ ,  $Zn^{2+}$ ,  $Cd^{2+}$ ,  $Al^{3+}$ ,  $Pb^{2+}$ ,  $Mn^{2+}$ ,  $Mn^{3+}$ .

7. An aqueous acid catalyst solution comprising a Pd(II) catalytic ion wherein said catalytic ion is present in amount sufficient to provide in the working strength 10 catalyst solution a concentration equivalent to about 10-500 mg/l of  $Pd^{2+}$  as  $PdCl_2$ , a stoichiometric excess of stannous salt, and a booster compound consisting of a soluble metal salt of which the cation is capable of forming a precipitate when contacted with the accelerator solution used in an electroless plating process employing a substrate which has been catalyzed in said catalyst solution, said booster compound being present in amount of about 0.1 mol/l up to 5 mol/l in the working strength solution.

8. An aqueous catalytic solution composition as defined in claim 7, wherein the booster compound is selected from the group consisting of  $Ca^{2+}$ ,  $Ba^{2+}$ ,  $Fr^{2+}$ ,  $Pb^{2+}$ ,  $Mg^{2+}$ ,  $Fe^{2+}$ ,  $Fe^{3+}$ ,  $Mn^{2+}$ ,  $Mn^{3+}$ ,  $Cu^{2+}$ ,  $Ni^{2+}$ ,  $Co^{2+}$ ,  $Cr^{3+}$ ,  $Cd^{2+}$ ,  $Zn^{2+}$ ,  $Pb^{2+}$ ,  $Al^{3+}$ .

\* \* \* \* \*